

1

3,276,839

**PROCESS OF TREATING SYNTHETIC POLYAMIDE TEXTILE MATERIALS WITH UNSUBSTITUTED POLYVALENT PHENOLS**

Georg Fröh, Wuppertal-Elberfeld, Germany, assignor to Vereinigte Glanzstoff-Fabriken A.G., Wuppertal-Elberfeld, Germany  
No Drawing. Filed Dec. 17, 1963, Ser. No. 331,130  
Claims priority, application Germany, Aug. 24, 1960,  
V 19,239

6 Claims. (Cl. 8—130.1)

This application is an continuation-in-part of application Serial No. 133,564 which was filed on August 24, 1961, and which is now abandoned.

The present invention is directed to a finishing and dyeing process for textile materials. More particularly, the subject invention relates to a finishing and dyeing process for threads, yarns, woven and knitted products which are made from synthetic polyamides.

Textile materials commonly are not only dyed but are also subjected to other finishing operations in order to improve the feel, appearance, and wearing ability of such materials. As an example, stockings which are made from polyamides, such as nylon, customarily are fixed with saturated steam or hot air to preserve their shape and to make the stockings soft to the touch. The softness and feel of such products can be improved even more by the use of particular softening agents. Organic swelling agents such as phenols or their aqueous solutions also improve the surface properties and increase the dye absorption of synthetic polyamides.

Although phenols improve certain properties of polyamide fabrics, it has been found that the presence of phenols in the dye baths often causes the color of the products to change under certain circumstances. This is true, for example, when ladies' hose are dyed with dispersion dyes such as water-insoluble Celliton dyes. The swelling action of the phenol which aids the dye absorption and improves the finish of a product, changes the color tone especially in the case of light colors such as are used in manufacturing ladies' hose. It has also been found that when the swelling of the textile products is begun with phenol and is finished with special vivifiers, the polyamide products lose their improved feel after repeated washings and become soft and ragged unless special wash resistant vivifiers are used.

It is an object of the present invention to provide a method of dyeing and finishing polyamide threads, yarns, and finished products in the presence of phenol which avoids the disadvantages outlined above.

Other objects of the invention will become apparent to those skilled in the art from the following detailed description.

In general, the present invention comprises the discovery that polyamide products having excellent properties can be produced if an unsubstituted polyvalent phenol and an aliphatic, anion-active compound is present in the finishing or dyeing bath and if the dyeing or finishing operation is carried out in an alkaline medium. The simultaneous presence of the phenol and the anion-active compound is of critical importance. If the textile materials are finished and dyed in successive steps, it is satisfactory to add the phenol and the aliphatic, anion-active compound only to the finishing bath. In this case the finishing operation prepares the textile material in such a manner that under ordinary dyeing conditions and without other special components being present, unobjectionable dyeing takes place and the finished product has a satisfactory feel and appearance.

Textile materials of polyamides which are dyed and finished in the presence of a phenol and an aliphatic,

2

anion-active compound in an alkaline medium not only have a uniform color but also demonstrate other valuable properties which distinguish such products from those treated only with a phenol. As an example, knitted articles of polyamide thread, particularly ladies' hose, when treated with a solution containing an unsubstituted polyvalent phenol and a hard soap at a pH of between 7 and 8 maintain their silklike feel and sheen after repeated washings. Furthermore, the appearance of such products

gives the impression that they have been treated with a softener. The danger of runs or snags in the case of knitted articles is also reduced by about one-third. Another manufacturing advantage which is realized with respect to stockings treated with the phenol and aliphatic, anion-active compound in an alkaline medium is that such stockings can be removed from their forms without difficulty and without the use of a particular softener. This advantage is not obtainable using phenol alone. For this reason the forming and fixing of the stockings may advantageously take place at the end of the manufacturing process as so-called postboarding. The possibility of combining the finishing and the dyeing steps, simplifies the manufacture of the products and offers economic advantages in comparison with prior art processes in which the woven or knitted articles are especially treated after dyeing in order to make them suitable for sale and wear.

Textile materials of synthetic polyamides which are finished or dyed in accordance with this invention have particularly advantageous properties when they are treated in the presence of ortho, meta and para-dihydroxy benzenes. The heat resistance of such materials is greatly increased. Threads of hexamethylene diamine-adipic acid-polycondensation products or of polycaprolactam which are finished in the presence of ortho-dihydroxy benzene demonstrate little, if any, decrease in tensile strength after heating for one hour at 200° C. In contrast, the tensile strength of untreated threads of the same type drop from 20% to 40% of the original tensile strength when subjected to the same heat conditions.

The method of carrying out the subject process is quite simple, especially when the finishing step is combined with the dyeing step. As an example, stockings made of polyamide threads, after presetting (steaming) and sewing, can be boiled for one hour in a solution of 10 grams per liter of phenol and 2.5 grams per liter of soap after which they are rinsed and dyed in a fresh bath. It is of advantage to combine both the dyeing and finishing operations by adding the phenol and aliphatic, anion-active compound to the dye bath. In this process the stockings are placed in the boiling treating bath for one hour, whereupon the stockings are rinsed and postboarded. The operation is carried out at an alkaline pH of between 7 and 8 which is the value of the solution if alkali metal salts of higher fatty acids are used as the aliphatic, anion-active compound. If another aliphatic, anion-active compound is used, such as a sulfated fatty alcohol, however, the proper pH value is obtained by adding a caustic sodium solution or soda to the treating agent.

The subject process is suitable for use in connection with dispersion dyes, 2:1 complex dyes, acid dyes, or substantive dyes. The use of such dyes in connection with polyamides is well known in the art.

Unsubstituted polyvalent phenols which can be used in the subject process include pyrocatechol, resorcinol, and hydroquinone which are also known as ortho, meta and para-dihydroxy benzenes, as well as pyrogallol and phloroglucinol. My preferred materials are ortho, meta and para-dihydroxy benzenes and the most preferred material is ortho-dihydroxy benzene.

70 A wide variety of aliphatic, anionic compounds can be used in the subject invention. Surface active agents are placed in one of three categories. These agents are

either anionic, cationic, or nonionic in character. If the elongated, low affinity portion of the molecule of the compound is included in the anion in aqueous solution, the substance is termed anion-active or anionic. The most common anionic aliphatic compounds are soaps such as the alkali metal salts of fatty acids. Such soaps are formed from fatty acids containing from 8 to 22 carbon atoms and preferably from 12 to 18 carbon atoms. The fatty acids can be both saturated and unsaturated. Illustrative examples of soaps would include sodium and potassium, laurate, myristate, palmitate, stearate, and oleate.

In addition to soaps, other satisfactory anion-active aliphatic compounds include sulfated fatty acids containing from 8 to 22 carbon atoms, and preferably from 12 to 18 carbon atoms, sulfated fatty alcohols containing from 8 to 22 carbon atoms, and preferably from 12 to 18 carbon atoms. In particular, such anion-active aliphatic compounds can include the sulfates or sulfonates of lauric acid, myristic acid, palmitic acid, stearic acid, oleic acid, dodecyl alcohol, tetradecyl alcohol, cetyl alcohol, octadecyl alcohol, oleyl alcohol, and mixtures thereof.

The following example is illustrative of the present invention.

*Example*

In this example 60 denier polyamide threads in the hank were dyed in a bath containing

10 grams per liter pyrocatechol (brenzcatechin)  
2.5 grams per liter hard soap (sodium stearate)  
1% Cibalan grey BL

The temperature of the bath was raised from room temperature to boiling and was held at this temperature for one hour. Thereafter the threads were rinsed in the customary manner. The threads had a silklike and substantial feel and also had improved heat resistance properties.

The subject finishing and dyeing process is generally applicable for textile materials of synthetic polyamides in any form. This includes threads and yarns on spools or hanks as well as woven or knitted materials made from synthetic polyamides.

The treatment time can vary over a wide range. In a preferred embodiment a dye bath having a temperature of from about 20 to 30° C. is brought to a boil in the course of from about 30 to 60 minutes, and is maintained at that temperature for from one-half to two hours.

As was pointed out above, the pH of the bath should be between about 7 and 8. If soaps are used as the treating agent, the pH of the bath will be maintained within this range without the addition of other materials. If sulfated alcohols, or the like, are used, however, it may be necessary to adjust the pH of the bath by the addition of caustic soda or some other alkaline compound.

The finishing or dye bath should contain from about

9 to 11 grams per liter of phenol, and preferably 10 grams per liter of phenol, and should contain from about 1.5 to 3 grams per liter of the anion-active aliphatic compound, and preferably from 2 to 2.5 grams per liter of the anion-active aliphatic compound.

As was pointed out above, the important features of the invention are the simultaneous use of the phenol and aliphatic, anion-active compound in treating synthetic polyamide, and the fact that the treating bath should be maintained at a pH of between about 7 and 8. Any anionic aliphatic compound bearing a hydrocarbon chain of from 8 to 22 carbon atoms, and preferably from 12 to 18 carbon atoms, can be used in the process. The hydrocarbon chain can either be saturated or olefinically unsaturated.

Obviously many modifications and variations of the invention as hereinbefore set forth may be made without departing from the spirit and scope thereof, and therefore only such limitations should be imposed as are indicated in the appended claims.

I claim:

1. A process for finishing textile materials of synthetic polyamides which comprises: contacting said polyamide with a boiling bath containing an unsubstituted polyvalent phenol and an aliphatic anion-active compound, at a pH of between about 7 and 8.

2. A process as in claim 1 wherein the polyamide is maintained in the boiling bath for about one-half to about two hours.

3. A process for finishing textile materials of synthetic polyamides which comprises: contacting said polyamide with a boiling bath containing an unsubstituted polyvalent phenol selected from the group consisting of pyrocatechol, resorcinol, hydroquinone, pyrogallol, and phloroglucinol, and an aliphatic anion-active compound selected from the group consisting of alkali metal salts of fatty acids containing from 8 to 22 carbon atoms, sulfated fatty acids containing from 8 to 22 carbon atoms, and sulfated fatty alcohols containing from 8 to 22 carbon atoms.

4. A process as in claim 3 wherein said bath contains from about 9 to 11 grams per liter of the phenol and from about 1.5 to about 3 grams per liter of the anion-active compound.

5. A process as in claim 3 wherein said bath contains about 10 grams per liter of the phenol and about 2 to 2.5 grams per liter of said anion-active substance.

6. A process as in claim 5 wherein said phenol is pyrocatechol and wherein said anion-active compound is stearic acid.

No references cited.

NORMAN G. TORCHIN, Primary Examiner.

J. C. CANNON, Assistant Examiner.